

May 30, 1967

J. TANZER

3,321,903

MOP YARN

Filed July 7, 1964

**FIG. 1**



**FIG. 2**



**FIG. 3**



INVENTOR  
JAY TANZER

BY *Frederick J. Butz*

ATTORNEY

# United States Patent Office

3,321,903

Patented May 30, 1967

1

3,321,903  
MOP YARN

Jay Tanzer, Wilmington, Del., assignor to E. I. du Pont de Nemours and Company, Wilmington, Del., a corporation of Delaware

Filed July 7, 1964, Ser. No. 380,898

9 Claims. (Cl. 57—140)

This invention relates to a sponge yarn and is more particularly directed to a sponge yarn made by sheathing a synthetic, bulky, textured, continuous filament fiber yarn core with cellulose sponge.

In the past, cellulosic sponge yarn has been made on a plied cotton fiber core, as shown in U.S. Patent 2,409,660 and U.S. Patent 2,600,143. Use of a cotton core gives a dense, stiff sponge yarn which is also less durable than its desired. Naturally, these properties are objectionable.

It has now been found that these deficiencies can be largely eliminated and, in fact, a superior yarn can be obtained by making the sponge yarn on a synthetic, textured, bulky, continuous filament yarn core. This synthetic yarn core contains a plurality of substantially continuous filaments which are individually convoluted into coils, loops and whorls at random intervals along their lengths. The yarn has a multitude of ring-like loops irregularly spaced along its surface. Such a yarn is illustrated in FIGURE 1 of the drawing, and is described in greater detail in Breen U.S. Patent 2,783,609.

A sponge sheath is anchored to this core by coagulating the sponge about the coils, loops and whorls of the yarn, as is shown in FIGURE 2 of the drawing, which presents a cross-section of a strand of sponge yarn of the invention. In this strand, the textured yarn core 1 is embedded in and sheathed with cellulose sponge 2. The bond formed in this way between the core and the sponge is durable and tenacious.

The sponge yarn of the invention is 40% more flexible<sup>1</sup> (wet) than comparable yarn made on a cotton core. This is surprising since Breen, in his P.S. Patent 2,783,609 says "The unmodified hand of fabrics made from the bulky yarn usually is stiffer than that of corresponding staple materials, making them more suitable for use in draperies, suits, overcoats, etc." Moreover, the sponge yarn of this invention has improved durability. It washes better and lasts longer than comparable yarn made on a cotton core.

In addition to all this, sponge yarn made with a textured yarn core does not exhibit blistering as does sponge yarn made on a cotton core. This blistering causes weak spots in the yarn which can, in turn, cause premature wear.

Synthetic, bulky, textured yarn suitable for use as a core material can be prepared according to the disclosures in Breen U.S. Patent 2,783,609, which is incorporated into and made a part of this specification to show materials and methods which can be used to make such cores. The yarn core can, for example, be made of nylon, cellulose acetate, vinyl or vinylidene resins, polyacrylonitrile, copolymers of acrylonitrile and other ethylenically unsaturated monomers, poly(ethylene terephthalate) polypropylene or high density polyethylene. Particularly preferred, however, because of its availability and the excellence of the product obtained with it, is a textured, bulky, poly(hexamethylene adipamide) yarn made according to the method of U.S. Patent 2,783,609.

Especially preferred is a texturized poly(hexamethylene adipamide) yarn made by placing three individual yarns

2

having 140 six-denier filaments each side-by-side and then processing them according to the method of U.S. Patent 2,783,609 to texturize them. These yarns are then twisted together to form a single yarn having a total denier of about 2700-2900.

The sponge material used to sheath the textured yarn core can be any of those known in the art. Suitable materials are described in U.S. Patents 2,280,022; 2,295,823; 2,329,239; 2,409,660; 2,600,143 and 3,068,545, and in patents cited therein. The sponge material is made with small Glauber's salt crystals, e.g., 70-80% of which will pass through a 20-mesh screen but will be held by a 30-mesh screen.

The sponge yarn itself is prepared by feeding the yarn core material into a sponge-forming mixture, prepared according to any of the patents mentioned above, as the mixture is extruded from a conventional sponge extruder fitted with a manifold and heads for extruding sponge yarn.

In such an extruder, the yarn core is fed into and through a nipple which extends into the sponge mix chamber. From the nipple, the yarn is passed through the sponge mix and out of the extruder through the center of an extrusion head. The yarn is passed out of the head as the sponge mixture is being extruded; this gives a strand of sponge-forming material having the textured yarn core embedded in it.

As it leaves the extruder, this strand of sponge-forming material is passed into a bath of aqueous saturated Glauber's salt solution, kept at or near its boiling point. This coagulates the material, melts the salt crystals and regenerates the cellulose. The resulting sponge yarn is then washed in water and dried. An end view of a sponge yarn produced in this way is presented in FIGURE 3 of the drawings.

The rate at which yarn is fed into the extruder and proper alignment of the yarn, is regulated by a series of driven rolls on the feed and the take-up ends of the yarn. It is, of course, important that the rate of yarn feed and the rate of mix extrusion be the same so that a satisfactory bond between the core and sponge is obtained.

For a smooth product, the core yarn should be kept at minimum tension as it passes through the extruder. Core yarn tensions which stretch the yarn appreciably give a "puckered" product, which in some cases may be desirable because the "puckers" help pick up grit when the sponge yarn is used in mopping operations.

The core yarn, when used to make a smooth product, should be kept at a tension of no more than about 10% of that required to break the yarn. When used to make a "puckered" product, it should be kept at a tension of about 75% to 80% of that required to break it.

The dimensions of the yarn core and the final product are a matter of choice. Diameter, denier, weight porosity—all are dictated by need and convenience. Variations on the basic theme of this invention can be composed by anyone skilled in this art.

The sponge yarn can, if desired, be modified to increase its aesthetic appeal by adding pigments, conventional plasticizers and softeners to the sponge forming mixture.

So that this invention will be more easily understood and readily practiced, the following example is submitted:

A sponge-forming mixture is prepared by thoroughly mixing, in a pug mill, 15 parts of a viscose-fiber composition, 77 parts of Glauber's salt ( $\text{Na}_2\text{SO}_4 \cdot 10\text{H}_2\text{O}$ ) crystals (which pass through a 20-mesh screen but are held by a 30-mesh screen), 8 parts of water and 0.2 part of a halogenated phthalocyanine green dispersion in water. The viscose-fiber composition contains 12.5% of alpha-cellulose, 2% flax fiber, 5.7% sodium hydroxide, 6% carbon bisulfide and 73.8% water.

<sup>1</sup> As measured on a Clark softness tester. In this test, three strands of sponge yarn are stapled together, side-by-side, with two staples  $\frac{1}{8}$  inch from the end of the yarn. The yarn is then wet with water and run through a set of washing machine wringers. These samples are then tested according to TAPPI Standard T-431m-60. Results are reported as stiffness.

A texturized poly(hexamethylene adipamide) yarn, previously described as being especially preferred, is fed as previously described, under a tension of about 10% of that required to break it, into this sponge-forming mixture as it is extruded from a  $\frac{1}{4}$  inch nozzle of a sponge yarn extruding machine. The resulting strand of sponge-forming mixture, having the texturized yarn embedded in it, is then coagulated and regenerated into cellulose sponge by immersing it for from 6-10 minutes in a boiling bath of 73% water, 26%  $\text{Na}_2\text{SO}_4 \cdot 10\text{H}_2\text{O}$  and 1% NaOH, washing it with water and then drying it.

The resulting smooth sponge yarn, having a diameter of about  $\frac{1}{4}$  inch, has a stiffness of about 40 as compared to about 67 for a cotton core yarn of the same diameter, and loses only 4.3% of its weight on washing for 72 hours in a washing machine, as compared with a 9.3% weight loss with a cotton core yarn of the same diameter.

This yarn, when made into a mop, can be washed and dried repeatedly, with no change in appearance or mopping ability. It is lighter in weight and has more water pickup than a corresponding cotton core yarn. Being more flexible, it is easier and more efficient to use, and water is squeezed from it with greater ease.

The claims are:

1. A mop yarn having improved flexibility and durability, said yarn comprising a strand of cellulosic sponge having a synthetic, textured, bulky yarn core, said yarn core comprising a plurality of substantially continuous filaments which are individually convoluted into coils, loops and whorls at random intervals along their lengths, said yarn core being characterized by the presence of a multitude of ring-like loops irregularly spaced along its surface.

2. A mop yarn according to claim 1 wherein the yarn core is made of nylon filaments.

3. A mop yarn according to claim 1 wherein the yarn core is made of poly(hexamethylene adipamide) filaments.

4. A mop yarn according to claim 3 wherein the yarn comprises three individual textured yarns having 140 six-

10 denier filaments each, the three individual yarns being twisted together to form a single yarn having a total denier of about 2700-2900.

15 5. A mop made of the yarn described in claim 1.

6. A process for the manufacture of cellulosic sponge yarn having improved flexibility and durability, said process comprising sheathing a synthetic, textured, bulky yarn core comprising a plurality of substantially continuous filaments which are individually convoluted into coils, loops and whorls at random intervals along their lengths, said yarn core being characterized by the presence of a multitude of ring-like loops irregularly spaced along its surface, with cellulosic sponge while maintaining said yarn core under a tension of no more than about 10% of that required to break the yarn core.

15 7. A process according to claim 6 wherein the yarn is made of nylon filaments.

8. A process according to claim 6 wherein the yarn is made of poly(hexamethylene adipamide) filaments.

9. A process for the manufacture of cellulosic sponge yarn having improved flexibility and durability, said process comprising sheathing a textured, bulky yarn core comprising a plurality of substantially continuous poly (hexamethylene adipamide) filaments which are individually convoluted into coils, loops and whorls at random intervals along their lengths, said yarn core being characterized by the presence of a multitude of yarn-like loops irregularly spaced along its surface, with cellulosic sponge while maintaining said yarn core under a tension of about 75-80% of that required to break the yarn core.

#### References Cited

#### UNITED STATES PATENTS

|    |           |         |        |        |
|----|-----------|---------|--------|--------|
| 35 | 2,409,660 | 10/1946 | Briggs | 15-229 |
|    | 2,600,143 | 6/1952  | Vaughn | 57-153 |
|    | 2,783,609 | 3/1957  | Breen  | 57-140 |

FRANK J. COHEN, Primary Examiner.

STANLEY N. GILREATH, J. PETRAKES,  
Assistant Examiners.